

July 12, 1960

G. M. DAVIS

2,945,051

METALLIC SALTS OF COMMERCIAL STEARIC ACID

Filed Oct. 19, 1955



*Fig. 1.*



*Fig. 2.*

INVENTOR.  
GERALD M. DAVIS,

BY

*Alexander T. Kardos.*

ATTORNEY.

# United States Patent Office

2,945,051

Patented July 12, 1960

1

2,945,051

## METALLIC SALTS OF COMMERCIAL STEARIC ACID

Gerald M. Davis, Clark Township, Union County, N.J., assignor to American Cyanamid Company, New York, N.Y., a corporation of Maine

Filed Oct. 19, 1955, Ser. No. 541,323

4 Claims. (Cl. 260—414)

The present invention relates to metallic stearates and more particularly to metallic salts or soaps of higher fatty acids of from about 12 to about 22 carbon atoms, which acids are known and sold in industry as "commercial fatty acids" and sometimes as "commercial stearic acids." More specifically, the present invention relates to magnesium, calcium and zinc soaps of higher fatty acids which are characterized by a relatively large crystal size. The invention includes the metallic stearate compositions and the methods of their preparation.

The greater portion of the metallic stearates of commerce are made from relatively cheap grades of "stearic acid" which are actually mixtures of higher fatty acids of from about 12 to about 22 carbon atoms and include both saturated and unsaturated acids. The solid acids and the hydrogenated fatty acids represent one group of these commercial fatty acids and normally contain (1) larger proportions of the saturated fatty acids and (2) smaller proportions of the unsaturated acids. This group of acids normally have iodine values of less than 20. On the other hand, the animal liquid acids, the vegetable liquid acids, the animal fatty acids and the vegetable fatty acids represent another large group of commercial fatty acids which normally contain (1) larger proportions of unsaturated acids and (2) smaller proportions of saturated acids. The members of this latter group normally have iodine values in excess of 20 and frequently up to as high as about 160 or more.

Metallic stearates such as zinc stearate prepared from acid mixtures of the former group of fatty acids are frequently used in lacquers, varnishes, printing inks and in surface coating compositions as flattening and sanding sealing agents and to provide covering power. When used for these purposes, a stearate composition having a relatively large average crystal size is preferred, with a minimum of smaller particles or fines of less than 1 micron average diameter. The flattening and covering efficiency, the sanding sealing properties and the viscosity characteristics of the lacquer would be considerably improved if zinc stearates having an average crystal size on the order of from about 1 to about 7 microns or larger were available with not more than about 5% by weight having a crystal size of less than about 1 micron. This has been established as desirable inasmuch as zinc stearate crystals in the range of from about 0.1 to about 1 micron in average diameter or slightly larger have been found to give poor flattening and sanding sealing properties and to form a gel in the lacquer, varnish, printing ink, or other material either during grinding or upon subsequent storage.

It is therefore a principal object of the present invention to provide metallic stearate having a relatively large crystal size and possessing improved efficiency as a flattening, covering and sanding sealing agent in surface coating compositions and exhibiting decreased gelling or thickening tendencies during grinding or working or on storage.

2

It has been found that the average crystal size of metallic soaps of commercial stearic acids is materially increased when acids of the first described group are used and when the metallic stearate is formed by a direct reaction of the fatty acids in a molten condition in a single continuous phase with an aqueous slurry of a hydroxide of the particular preferred metal.

Metallic stearates have formerly been prepared normally by reacting the selected fatty acid with an alkali metal hydroxide and then reacting the resulting alkali metal stearate with a metallic salt whereby the metallic stearate, which is formed by metathesis, precipitates out and is separated, filtered, washed and dried.

Other methods have been employed wherein the fatty acids have been present in an emulsified or dispersed condition, such as an aqueous emulsion, and the metallic soap which precipitated out was collected, filtered, washed and dried.

These methods normally produce metallic stearates having relatively small crystal size such as is shown in Figure 1. The improved methods of the present invention produce a product having a much larger crystal size such as illustrated in Figure 2 of the drawing.

The improved methods of the present invention are therefore distinguished from the methods of the prior art in (1) the fact that the metallic stearates are formed by a direct reaction of the fatty acids and the hydroxide of the desired metal without going through any intermediate stages involving the preparation of alkali metal stearates and (2) the fact that the fatty acid mixture is present in a molten condition in a single continuous phase and not in an emulsified or dispersed polyphase system.

In general, an aqueous slurry of the hydroxide is employed and is normally added slowly with gentle agitation to the fatty acid mixture which has previously been heated so that it is in a molten condition.

The molten condition of the fatty acid mixture may be obtained by applying heat directly to the mixture of solid fatty acids until it melts but it is preferred to add the solid fatty acids to water and to heat the same until the fatty acid mixture melts and floats as a single continuous phase or layer on top of the water.

In the event that a gentle agitation is used during the heating of the fatty acid, such should not be enough to form an emulsion or to intermix the water and the fatty acid to any substantial degree. No emulsion agent should be present which would tend to create either a temporary emulsion or a permanent emulsion.

The slurry of the particular hydroxide is added slowly to the molten fatty acid and the metallic stearate precipitates out in the usual fashion as known in the art and is then separated, filtered, washed and dried by procedures known in the art.

The invention will be further described by reference to the following examples which set forth the specific embodiments of the present invention. These embodiments, however, are merely illustrative and are not to be construed as limitative of the present invention.

### Example 1

A sodium stearate soap solution was prepared by adding 127 lbs. of sodium hydroxide to 936 gallons of hot water at a temperature of approximately 70-75° C. 800 lbs. of "Emersol 110" (2% myristic acid, 48% palmitic acid, 39% stearic acid, 10% oleic acid and 1% linoleic acid) was then added to the sodium hydroxide solution and the volume of the reaction mixture was adjusted to 1155 gallons in order to secure the desired concentration. The pH of this solution was approximately 11-11.5 and the temperature of the final solution was approximately 70° C.

300 lbs. of zinc sulfate (36% zinc) was dissolved in 2140 gallons of hot water at a temperature of approximately 60-70° C. 1.2 lbs. of concentrated hydrochloric acid (C.P.) was added to this solution which was then diluted to 2996 gallons for the desired concentration. The pH of this solution was determined to be 3.0.

2322 gallons of hot water at approximately 67° C. was run into a precipitating tank. The sodium stearate soap solution and the zinc sulfate solution were then simultaneously run into the warm water. Measurements of the pH were taken continuously and the pH was controlled to 6.5-6.7. A small amount of zinc sulfate was then added to adjust the final pH to 6.5.

The precipitate of zinc stearate was then separated by a filtering operation wherein the wash water comprised softened water at a temperature above 22° C. The drying took place with air heated to a temperature 103°-105° C. during the earlier part of the drying and 100° C. during the later part of the drying.

The final product has the following analysis:

|                   |         |      |
|-------------------|---------|------|
| Moisture          | percent | 0.6  |
| Water soluble ash | do      | 0.5  |
| ZnO content       | do      | 14.6 |
| Acid No.          |         | 1.2  |
| Percent CaO       |         | 0.02 |
| Percent Fe        | p.p.m.  | 30   |

The zinc stearate resulting from this method of substantially simultaneously adding the sodium stearate solution and the zinc sulfate solution was a relatively fine crystalline product and is illustrated in Figure 1. Such a product was satisfactorily used as a mold lubricant but was not acceptable as a flattening or sanding sealing agent.

#### Example 2

400 grams of zinc sulfate ( $ZnSO_4 \cdot H_2O$ ) was dissolved in 2000 grams of water at room temperature. 179.5 grams of 100% sodium hydroxide (dissolved) was added to the zinc sulfate solution with slow agitation.

100 grams of Hyfac 400 (a hydrogenated fatty acid of a relatively cheap rubber grade having high color (70Y/14R—5.25" S.C.) and containing 1% lauric acid, 3% myristic acid, 28% palmitic acid, 63% stearic acid and 5% oleic acid) (Iodine value—Wij—10) was melted in 16,000 grams of hot water maintained at a temperature between 65° and 70° C. Slow agitation was used and was not sufficiently strong as to emulsify or disperse the fatty acid which remained for the most part in a separate layer distinct from the hot water layer.

The zinc hydroxide slurry formed by the reaction of the zinc sulfate and the sodium hydroxide was then added to the melted fatty acid with slow agitation and the temperature was maintained between 65° and 70° C. The zinc stearate precipitated out, was separated and filtered, washed and then dried at a temperature of about 100° to 105° C. for about 45 minutes.

The resulting zinc stearate had the following properties:

|                                               |
|-----------------------------------------------|
| 15.68% total ash                              |
| 15.28% washed ash                             |
| 0.40% water soluble ash                       |
| 1.43% moisture and volatile matter at 105° C. |
| 7.45 apparent density (lbs./cu. ft.)          |
| 1.68 acid value (mgm. KOH)                    |
| 6000 film area (sq. cm./g.)                   |

The zinc stearate resulting from this method of preparation was a relatively coarse crystalline product and is illustrated in Figure 2. Such a product was satisfactorily used as a flattening and sanding sealing agent.

#### Example 3

200 grams of zinc sulfate ( $ZnSO_4 \cdot H_2O$ ) was dissolved in 1200 grams of water at room temperature. 85 grams of 100% sodium hydroxide (dissolved) was added to the zinc sulfate solution with slow agitation.

500 grams of Hyfac 410 (a hydrogenated tallow fatty acid having a lower color (30Y/5R—5.25" S.C.) than Hyfac 400 and containing 1% lauric acid, 3% myristic acid, 28% palmitic acid, 63% stearic acid and 5% oleic acid) (Iodine value—7) was melted in 16,000 grams of hot water maintained at a temperature between 65° and 70° C. Slow agitation was used and was not sufficiently strong as to emulsify or disperse the fatty acid which remained for the most part in a separate layer distinct from the hot water layer.

10 The zinc hydroxide slurry formed by the reaction of the zinc sulfate and the sodium hydroxide was then added to the melted fatty acid with slow agitation and the temperature was maintained between 65° and 70° C.

15 The zinc stearate precipitated out, was separated and filtered, washed and then dried at a temperature of about 100° to 105° C. for about 45 minutes.

16 The resulting zinc stearate had the following properties:

|    |                                               |
|----|-----------------------------------------------|
| 20 | 15.48% total ash                              |
|    | 15.10% washed ash                             |
|    | 0.38% water soluble ash                       |
|    | 0.80% moisture and volatile matter at 105° C. |
| 25 | 8.0 apparent density (lbs./cu. ft.)           |
|    | 0.84 acid value (mgm. KOH)                    |
|    | 5250 film area (sq. cm./g.)                   |

30 The zinc stearate resulting from this method of preparation was a relatively coarse crystalline product and was approximately similar in size to the crystals illustrated in Figure 2. (Majority of crystals between 1 and 7 microns.) Such a product was satisfactorily used as a flattening and sanding sealing agent.

#### Example 4

35 200 grams of zinc sulfate ( $ZnSO_4 \cdot H_2O$ ) was dissolved in 1200 grams of water at room temperature. 85 grams of 100% sodium hydroxide (dissolved) was added to the zinc sulfate solution with slow agitation.

40 500 grams of Hyfac 420 (a hydrogenated tallow fatty acid having a color 4Y/0.4R—5.25" S.C. and containing 3% myristic acid, 29% palmitic acid, 65% stearic acid and 3% oleic acid) (Iodine value—3) was melted in 16,000 grams of hot water maintained at a temperature between 65° and 70° C. Slow agitation was used and was not sufficiently strong as to emulsify the fatty acid which remained for the most part in a separate layer distinct from the hot water layer.

45 The zinc hydroxide slurry formed from the reaction of the zinc sulfate and the sodium hydroxide was then added to the melted fatty acid and the temperature was maintained between 65° and 70° C. The zinc stearate precipitated out, was separated and filtered, washed and then dried at a temperature of about 100° to 105° C. for about 45 minutes.

50 The resulting zinc stearate had the following properties:

|    |                                               |
|----|-----------------------------------------------|
| 55 | 15.75% total ash                              |
|    | 15.20% washed ash                             |
|    | 0.55% water soluble ash                       |
| 60 | 1.08% moisture and volatile matter at 105° C. |
|    | 8.4 apparent density (lbs./cu. ft.)           |
|    | 1.20 acid value (mgm. KOH)                    |
|    | 5500 film area (sq. cm./g.)                   |

65 The zinc stearate resulting from this method of preparation was a relatively coarse crystalline product similar to that illustrated in Figure 2. Such a product was satisfactorily used as a flattening and sanding sealing agent.

#### Example 5

70 200 grams of zinc sulfate ( $ZnSO_4 \cdot H_2O$ ) was dissolved in 16,000 grams of water and heated to a temperature between 65° and 70° C. 500 grams of Hyfac 410 (Iodine value—5) was slowly added to the hot zinc sulfate solution and slowly agitated until it was molten. 85

grams of 100% sodium hydroxide was then added to the hot fatty acid and zinc sulfate mixture.

The zinc stearate precipitated out, was separated and filtered, washed and then dried at a temperature of about 100° to 105° C. for about 45 minutes.

The resulting zinc stearate had the following properties:

16.05% total ash  
15.50% washed ash  
0.55% water soluble ash  
1.03% moisture and volatile matter at 105° C.  
8.1 apparent density (lbs./cu. ft.)  
1.40 acid value (mgm. KOH)  
5500 film area (sq. cm./g.)

The zinc stearate resulting from this method of preparation was a relatively coarse crystalline product having a particle size ranging from about 1 micron up to about 7 microns with less than 5% by weight less than about 1 micron.

#### Example 6

200 grams of zinc sulfate ( $ZnSO_4 \cdot H_2O$ ) was dissolved in 1200 grams of water at room temperature. 85 grams of 100% sodium hydroxide (dissolved) was added to the zinc sulfate solution with slow agitation.

500 grams of Hyfac 430 (a hydrogenated fish oil fatty acid containing 4% myristic acid, 32% palmitic acid, 22% stearic acid, 23% arachidic acid, 13% behenic acid and 6% oleic acid) (Iodine value—10) was melted in 16,000 grams of hot water maintained at a temperature between 65° and 70° C. Slow agitation was used and was not sufficiently strong as to emulsify the fatty acid which remained for the most part in a separate layer distinct from the hot water layer.

The zinc hydroxide slurry formed from the reaction of the zinc sulfate and the sodium hydroxide was then added to the melted fatty acid with slow agitation and the temperature was maintained between 65° and 70° C. The zinc stearate precipitated out, was separated and filtered, washed and then dried at a temperature of about 100° to 105° C. for about 45 minutes.

The resulting zinc stearate had the following properties:

17.88% total ash  
14.80% washed ash  
3.08% water soluble ash  
0.50% moisture and volatile matter at 105° C.  
8.0 apparent density (lbs./cu. ft.)  
1.68 acid value (mgm. KOH)  
5250 film area (sq. cm./g.)

The zinc stearate resulting from this method of preparation was a relatively coarse crystalline product and was in approximately the same particle size as the product illustrated in Figure 2. Such a product was satisfactorily used as a flattening and sanding sealing agent.

#### Example 7

400 grams of zinc sulfate ( $ZnSO_4 \cdot H_2O$ ) was dissolved in 2000 grams of water at room temperature. 180 grams of 100% sodium hydroxide (dissolved) was added to the zinc sulfate solution with slow agitation.

1000 grams of Emersol 110 (a single pressed fatty acid containing 2% myristic acid, 48% palmitic acid, 39% stearic acid, 10% oleic acid and 1% linoleic with an Iodine value of 15) was melted in 16,000 grams of hot water maintained at a temperature between 65° and 70° C. Slow agitation was used and was not sufficiently strong as to emulsify the fatty acid which remained for the most part in a separate layer distinct from the hot water layer.

The zinc hydroxide slurry formed from the reaction of the zinc sulfate and the sodium hydroxide was then added to the melted fatty acid with gentle agitation and the temperature was maintained between 65° and 70° C. The zinc stearate precipitated out, was separated and fil-

75

tered, washed and then dried at a temperature of about 100° to 105° C. for about 45 minutes.

The resulting zinc stearate had the following properties:

15.88% total ash  
15.38% washed ash  
0.50% water soluble ash  
1.30% moisture and volatile matter at 105° C.  
7.4 apparent density (lbs./cu. ft.)  
1.68 acid value (mgm. KOH)  
6000 film area (sq. cm./g.)

The zinc stearate resulting from this method of preparation was a relatively coarse crystalline product and is illustrated in Figure 2. Such a product was satisfactorily used as a flattening and sanding sealing agent.

#### Example 8

165 grams of calcium chloride ( $CaCl_2 \cdot H_2O$ ) was dissolved in 1200 grams of water at room temperature.

20 93 grams of 100% sodium hydroxide (dissolved) was added to the calcium chloride solution with slow agitation.

25 600 grams of Hyfac 400 was melted in 16,000 grams of hot water at a temperature maintained between 65° and 70° C. Slow agitation was used which was not sufficiently strong as to emulsify or disperse the fatty acid which remained for the most part in a separate layer distinct from the hot water layer.

30 The calcium hydroxide slurry formed by the reaction of the calcium chloride of the sodium hydroxide was then added with slow agitation to the melted fatty acid and the temperature was maintained between 65° and 70° C. The calcium stearate precipitated out, was separated and filtered, washed and then dried at a temperature of about 35 100° to 105° C. for about 45 minutes.

The resulting calcium stearate had the following properties:

9.28% total ash  
9.20% washed ash  
40 0.08% water soluble ash  
2.9% moisture and volatile matter at 105° C.  
9.2 apparent density (lbs. per cu. ft.)  
3.64 acid value (mgm. KOH)  
Percent chloride—slight trace

45 The calcium stearate resulting from this method of precipitation was a relatively coarse crystalline product having a particle size which was well above an average of 1 micron, with several particles being noted as about 7-8 microns across. Such a product was satisfactorily used in waterproofing compositions wherein the larger plate-like crystals provided for more even spreading. The product showed no tendencies to form a gel in coating material either during grinding or upon subsequent storage.

#### Example 9

50 165 grams of calcium chloride ( $CaCl_2 \cdot H_2O$ ) and 600 grams of Hyfac 410 were dissolved in 16,000 grams of water at a temperature of about 65-70° C. 93 grams of 100% sodium hydroxide (dissolved) was added to the mixture with slow agitation. The calcium stearate precipitated out, was separated and filtered, washed, then dried at a temperature of about 100 to 105° C. for about 45 minutes.

55 The resulting calcium stearate had the following properties:

7.28% total ash  
7.20% washed ash  
0.08% water soluble ash  
70 2.5% moisture and volatile matter at 105° C.  
7.5 apparent density (lbs. per cu. ft.)  
1.56 acid value (mgm. KOH)  
Percent chloride—slight trace

The calcium stearate resulting from this method of

precipitation was a relatively coarse crystalline product and is similar to that illustrated in Figure 2. Such a product was satisfactorily used in coating compositions and showed no tendencies to form a gel either during grinding or upon subsequent storage.

*Example 10:*

165 grams of calcium chloride ( $\text{CaCl}_2 \cdot \text{H}_2\text{O}$ ) was dissolved in 1200 grams of water at room temperature. 93 grams of 100% sodium hydroxide (dissolved) was added to the calcium chloride solution with slow agitation.

600 grams of Emersol 130 (a triple-pressed fatty acid containing 1% myristic acid, 50% palmitic acid, 47% stearic acid and 2% oleic acid) was melted in 16,000 grams of hot water at a temperature maintained between 65° and 70° C. Slow agitation was used which was not sufficiently strong as to emulsify or disperse the fatty acid which remained for the most part in a separate layer distinct from the hot water layer.

The calcium hydroxide formed by the reaction of the calcium chloride of the sodium hydroxide was then added to the melted fatty acid and the temperature was maintained between 65° and 70° C. The addition is made slowly with slow agitation. The calcium stearate precipitated out, was separated and filtered, washed and then dried at a temperature of about 100 to 105° C. for about 45 minutes.

The resulting calcium stearate had the following properties:

9.55% total ash  
9.50% washed ash  
0.05% water soluble ash  
2.3% moisture and volatile matter at 105° C.  
7.4 apparent density (lbs. per cu. ft.)  
1.12 acid value (mgm. KOH)  
Percent chloride—slight trace

The calcium stearate resulting from this method of precipitation was relatively coarse crystalline product and was satisfactorily used in coating compositions. It possessed excellent covering power and showed no gelling or thickening action.

*Example 11:*

100 grams of hydrated lime was dissolved in 1200 grams of hot water at about 65-70° C.

600 grams of Hyfac 420 was melted in 16,000 grams of hot water at a temperature maintained between 65° and 70° C. Slow agitation was used which was not sufficiently strong as to emulsify or disperse the fatty acid which remained for the most part in a separate layer distinct from the hot water layer.

The lime slurry was then slowly with gentle agitation added to the melted fatty acid and the temperature was maintained between 65° and 70° C. The calcium stearate precipitated out, was separated and filtered and then dried at a temperature of about 100 to 105° C. for about 45 minutes.

The resulting calcium stearate had the following properties:

10.65% total ash  
10.60% washed ash  
0.05% water soluble ash  
1.9% moisture and volatile matter at 105° C.  
10.0 apparent density (lbs. per cu. ft.)  
2.24 acid value (mgm. KOH)  
Percent chloride—slight trace

The calcium stearate resulting from this method of precipitation was a relatively coarse crystalline product having a particle size which was well above an average diameter of 1 micron, with several particles being noted as about 7-8 microns diameter. Such a product was satisfactorily used in a waterproofing composition and

showed no tendencies to form a gel either during grinding or upon subsequent storage.

*Example 12:*

100 grams of hydrated lime was added to 16,000 grams of water at 65-70° C. temperature.

600 grams of Hyfac 430 was melted and added slowly to the dilute lime slurry with slow agitation.

The calcium stearate precipitated out, was separated and filtered and then dried at a temperature of about 100 to 105° C. for about 45 minutes.

The resulting calcium stearate had the following properties:

10.80% total ash  
10.70% washed ash  
0.10% water soluble ash  
2.63% moisture and volatile matter at 105° C.  
13.50 apparent density (lbs. per cu. ft.)  
7.00 acid value (mgm. KOH)  
0.05% chlorides

The calcium stearate resulting from this method of precipitation was a relatively coarse crystalline product and was used satisfactorily in water proofing paper, textiles, cordage, wood, cement, plaster, asbestos, rockwool, and various building materials. It showed no tendencies to form a gel or thicken either during grinding or upon subsequent storage.

*Example 13:*

238 grams of magnesium sulfate ( $\text{MgSO}_4$ ) was dissolved in 1000 grams of water at room temperature. 75 grams of solid 100% sodium hydroxide was dissolved in 500 grams of water and the two solutions were mixed together, thereby forming a freshly prepared magnesium hydroxide slurry.

500 grams of Hydrofol 405 (a commercial fatty acid containing 1.5%  $\text{C}_{14}$ , 28.0%  $\text{C}_{16}$  and 70.5%  $\text{C}_{18}$  with 6% of the acids being unsaturated and 94% being saturated and an Iodine value (Wijs) of 6) was melted in 16,000 grams of hot water at a temperature of about 75° C.

The magnesium hydroxide slurry was slowly added with gentle agitation to the melted fatty acid and the temperature was maintained about 75° C. The magnesium hydroxide precipitated out, was separated and filtered, washed and then dried at a temperature of about 75° C. for about 15 hours.

The resulting magnesium stearate had the following properties:

8.02% total ash  
6.88% washed ash  
1.14% water soluble ash  
0.65% moisture and volatile matter at 105° C.  
4.06 acid value (mgm. KOH)

55 The magnesium stearate resulting from this method of preparation was a relatively coarse crystalline product and apparently existed in plate-like structures having less of a tendency to ball up, gel or thicken.

Although I have described but a few specific examples of my inventive concept, I consider the same not to be limited thereby nor to the specific substances mentioned therein, but to include various other compounds of equivalent constitution as set forth in the claims appended hereto. It is to be understood, of course, that any suitable changes, modifications and variations may be made without departing from the scope and spirit of the invention.

What I claim is:

1. A method of producing a coarsely crystalline metallic soap composition having an average crystal size of from about 1 to 7 microns in diameter with not more than 5% less than 1 micron in diameter from a mixture of commercial fatty acids of from 12 to 22 carbon atoms containing less than 20% by weight of unsaturated fatty acids and having an iodine value of less than 20 which

comprises supporting a continuous phase layer of said mixture of fatty acids in molten condition on an underlying body of a hot aqueous liquid, reacting therewith an aqueous slurry of a hydroxide of a metal from the group consisting of magnesium, calcium and zinc while maintaining the fatty acid layer distinct from the underlying aqueous layer and thereby precipitating a soap of said metal and said mixture of fatty acids and washing and drying the soap so produced.

2. A method of producing a coarsely crystalline zinc soap composition having an average crystal size of from about 1 to 7 microns in diameter with not more than 5% less than 1 micron in diameter from a mixture of commercial fatty acids of from 12 to 22 carbon atoms containing less than 20% by weight of unsaturated fatty acids and having an iodine value of less than 20 which comprises supporting a continuous phase layer of said mixture of fatty acids in molten condition on an underlying body of a hot aqueous liquid, reacting therewith an aqueous slurry of zinc hydroxide while maintaining the fatty acid layer distinct from the underlying aqueous layer and thereby precipitating the zinc soap of said mixture of fatty acids and washing and drying the soap so produced.

3. A coarsely crystalline metallic soap selected from the group consisting of the magnesium, calcium and zinc

soaps of commercial fatty acids of from 12 to 22 carbon atoms containing less than 20% by weight of unsaturated fatty acids and having an iodine value of less than 20, said soap being characterized by an average crystal size of from about 1 to about 7 microns in diameter with not more than about 5% by weight having diameters less than 1 micron and by an absence of gel-forming tendencies in coating compositions.

4. A coarsely crystalline zinc soap of a mixture of commercial fatty acids of from 12 to 22 carbon atoms containing less than 20% of unsaturated fatty acids and having an iodine value of less than 20, said soap being characterized by an average crystal size of from about 1 to about 7 microns in diameter with not more than 5% by weight having diameters less than 1 micron and by an absence of gel-forming tendencies when the soap is incorporated into a surface coating composition.

References Cited in the file of this patent

UNITED STATES PATENTS

|           |              |       |               |
|-----------|--------------|-------|---------------|
| 2,466,925 | Brauner      | ----- | Apr. 12, 1949 |
| 2,650,932 | Kebrick      | ----- | Sept. 1, 1953 |
| 2,809,121 | Davis et al. | ----- | Oct. 8, 1957  |

OTHER REFERENCES

Fisher: Soaps and Proteins, 1921, pages 10 and 26.